

No. 788,612.

PATENTED MAY 2, 1905.

T. H. SYMINGTON.

CORE FOR MAKING HOLLOW CASTINGS.

APPLICATION FILED DEO. 7, 1903.

2 SHEETS—SHEET 1.

FIG. 1.



FIG. 2.



WITNESSES

John M. Morris  
Denya Mathews.

INVENTOR

T. H. Symington

Stewart & Stewart  
ATTYS.

No. 788,612.

PATENTED MAY 2, 1905.

T. H. SYMINGTON.

CORE FOR MAKING HOLLOW CASTINGS.

APPLICATION FILED DEC. 7, 1903.

2 SHEETS—SHEET 2.

FIG. 3.



FIG. 4.



FIG. 5.



WITNESSES

John Morris  
Deniza Matthews

INVENTOR

T. H. Symington

by

Stewart & Stewart ATTYS.

## UNITED STATES PATENT OFFICE.

THOMAS HARRISON SYMINGTON, OF BALTIMORE, MARYLAND, ASSIGNOR  
TO THE T. H. SYMINGTON COMPANY, A CORPORATION OF DELA-  
WARE.

## CORE FOR MAKING HOLLOW CASTINGS.

SPECIFICATION forming part of Letters Patent No. 788,612, dated May 2, 1905.

Application filed December 7, 1903. Serial No. 184,111.

*To all whom it may concern:*

Be it known that I, THOMAS HARRISON SYMINGTON, a citizen of the United States of America, residing at Calvert Building, Baltimore city, Maryland, (and whose post-office address is Calvert Building, Baltimore city, Maryland,) have invented certain new and useful Improvements in Cores for Making Hollow Castings, of which the following is a specification.

My invention relates to a core used for casting, and is specially designed for the manufacture of a cheap and practical core for casting journal-boxes for railroad-cars.

In the casting of journal-boxes heretofore difficulty has been experienced in getting a green core to stand up during handling and casting. This may be accomplished by baking the whole core; but this is difficult and expensive. I have invented a core which is entirely practical and at the same time easy to handle, strong, and cheap to construct.

My invention consists of a core for casting journal-boxes the lower portion of which is of dry sand and is suspended from a suitable support, the upper portion of which is of green sand and is supported by the dry part, thus forming a strong and comparatively cheap core for a complicated casting.

In the drawings, Figure 1 is a vertical section of a core-box in which the dry core is made. Fig. 2 is a vertical section of the core-box in which the green core is made superimposed upon the dry core. Fig. 3 is a plan of the completed core. Fig. 4 is a side elevation of the completed core. Fig. 5 is a vertical longitudinal section of the mold with the core in full elevation and showing the casting in section.

Referring to Fig. 1 of the drawings, 1 is a core-box in which is molded a sand core 2, and when made a staple 3 is embedded in it.

This core 2 when molded is removed from its core-box and baked in an oven, so as to give it the desired degree of hardness and strength so that it may be suspended from a rod 5 when placed in the green-sand-core box and in the mold and also so that it may safely sustain the weight of the green-sand core which is built up upon it.

Referring to Fig. 2 of the drawings, 4 is the green-sand-core box, in the lower part of which the dry-sand core 2 is suspended from the rod 5, which passes through the core-box and the two ends of which rest in the openings in either end of the core-box. 6 is a dry-sand core made in another core-box and baked and set up in a suitable groove in the core-box, so as to be incorporated into the core. The vacant part of the core-box is then packed with green sand occupying the space marked 7 in Figs. 2, 3, 4, and 5, and the core is complete, as shown in Figs. 3 and 4. The core is then removed from the core-box and placed in the mold 8, as shown in Fig. 5, and a box cast within the mold and around the core, as shown in Fig. 5 at 9.

Having thus described my invention, what I claim, and desire to secure by Letters Patent, is—

A core for casting composed of a section of baked sand, a hanger embedded in said baked portion, a support co-operating with the hanger to support the baked section and a section composed of green sand superimposed upon the baked sand.

Signed by me at Baltimore city, Maryland, this 9th day of November, 1903.

THOMAS HARRISON SYMINGTON.

Witnesses:

T. BAYARD WILLIAMS,  
THORVALD A. LEE.